

## UNITED STATES PATENT OFFICE

AUGUSTUS B. KINZEL, OF NEW YORK, N. Y., ASSIGNOR TO ELECTRO METALLURGICAL COMPANY, A CORPORATION OF WEST VIRGINIA

## SURFACE-HARDENED MATERIAL AND METHOD FOR PRODUCING THE SAME

No Drawing.

Application filed July 28, 1927. Serial No. 209,184.

My invention relates to the surface hardening of members composed of ferrous metal, the hardening being effected by the action of nitrogen-containing compounds, for example 5 ammonia.

The hardening effect produced by heating ferrous metal in contact with ammonia and other nitrogenous compounds is known. It is also known that a desirable degree of hardness can only be obtained by this method 10 when the ferrous metal treated contains certain alloying elements, and when such alloying elements are present in critical amount. Acceptable hardening has been obtained 15 when the alloying element used was aluminum.

Aluminum is not a desirable alloying element in steel, as it tends to produce oxide inclusions and other defects which impair the 20 quality of the steel, particularly with respect to fatigue-resistance. The lack of desirable properties in those aluminum steels in which a hard surface layer can be developed by nitrogenizing seriously limits the 25 commercial usefulness of structures made therefrom.

My invention provides means for making a hard and strong nitride coating on ferrous metals without introducing into the metal an 30 undesirable constituent that will impair its properties.

I have discovered when aluminum is incorporated in ferrous metals only at the surface of the material where it is to be utilized 35 to produce the desired hard and strong nitrogenized structure that the undesirable effect of aluminum in the core is avoided.

I provide a steel with an aluminized surface layer containing a content of aluminum 40 such that a hardened layer will result when the steel is nitrogenized. The steel may be aluminized in any desired manner, but I prefer to heat the steel in contact with aluminum powder under neutral or reducing conditions 45 at a temperature of about 500° to 800° C. I have obtained satisfactory results when the steel was treated with aluminum for one-half to two hours at 550° C., but other temperatures and times may be used. If, by chance 50 the concentration of aluminum in the surface

becomes too great, I may reduce it to the desired value by soaking the steel at a suitable temperature, as for example about 900° C.

The surface-aluminized steel is then heated to about 500° to 580° C. in the presence of a 55 substance, such as ammonia, that yields nitrogen to the material. This treatment provides a hard nitrogenized compound of the kind described above only as a surface layer and the properties of the core of the material 60 will not be detrimentally affected. The nitrogenization preferably is carried out at a temperature not materially above 580° C., and under these conditions there is no serious embrittling of the interior portions of the 65 member treated.

My process is applicable to iron, steel and all ferrous alloys that are capable of absorbing a coating of aluminum, and may be applied to steel containing an amount of aluminum less than the critical amount necessary 70 to produce the desired hard coating. For example, I place a low carbon steel containing 12% chromium in a closed furnace chamber in a mixture of aluminum and aluminum oxide. The chamber and its contents are heated to a temperature of about 500° C., in an atmosphere of hydrogen for about two hours and then the steel is transferred with or without cooling to another furnace and 75 maintained in the latter furnace in an atmosphere of ammonia at 510° C. After treating in the latter furnace, the steel acquires a thin, hard, tough coating corresponding to about 900 of the Brinell scale. The hardness 80 of a carbon steel containing .35% carbon when aluminized and treated in accordance with my invention was likewise increased to about 900 Brinell. For most practical purposes, a hardness greater than 700 Brinell 85 is desired and a hardness of at least 900 Brinell is preferred.

The treated article resulting from my process has a core or foundation consisting of steel or alloy steel and a thin homogeneous 95 surfacing material comprising aluminum and nitrogen that provides a hard, strong coating. The core of the article contains either no aluminum or aluminum in a concentration so small that the core material is not detri- 100

mentally affected to the degree that it is when the core contains aluminum throughout in an amount sufficient to produce the desired hard nitrogenized surface layer.

5 Although I have described certain specific modifications of my invention, other modifications may be made without departing from the spirit thereof. Therefore, I desire to be limited only by the prior art and 10 by the invention as defined in the annexed claims.

I claim:

1. The method of hardening ferrous material which comprises enriching the material 15 in its surface layer with aluminum and then heating the material to about 510° C. in the presence of ammonia.

2. The method of hardening ferrous material which comprises heating the same in 20 contact with aluminum at a temperature sufficient to provide a surface layer enriched with aluminum and then heating the material in the presence of a substance that yields nitrogen.

25 3. The method of hardening ferrous material which comprises heating the same in contact with aluminum at a temperature sufficient to provide a surface layer comprising aluminum and then heating the material 30 to a temperature not exceeding 580° C. in the presence of a substance that yields nitrogen, said temperature being sufficient to nitrogenize the ferrous material.

4. The method of hardening ferrous material which comprises heating the same in 35 contact with aluminum at a temperature sufficient to provide an aluminized coating thereon and then heating the material to about 510° C. in the presence of ammonia.

40 5. The method of hardening ferrous materials which comprises heating the same with aluminum to about 550° C. so as to form a surface layer enriched with aluminum and then subjecting the material to a temperature 45 of about 510° C. in the presence of ammonia.

6. The method of hardening the surface of a ferrous material which comprises providing an aluminized coating on the material, the aluminum in said coating being of such concentration that a hard structure of complex nitrides will be formed only in the surface 50 layer when it is subjected to a substance that yields nitrogen and then heating the material to 500° to 580° C. in said substance.

55 7. An article comprising a core of ferrous material and a surface layer of a comparatively harder material, the surface layer of said article comprising a body of said ferrous material that has been aluminized and then 60 treated to form a hard nitrogenized body.

8. An article comprising a core of ferrous material and an aluminized surface layer of said ferrous material, said surface layer comprising a compound of nitrogen.

65 9. An article comprising a core of ferrous

material and a surface layer of aluminized core material, said surface layer being harder than said core and comprising a compound of nitrogen.

10. An article composed of ferrous metal having a hard surface layer containing aluminum and nitrogen, and a softer interior portion having a lower content of aluminum.

11. An article comprising a core containing a substantial amount of chromium, said article having an aluminized nitrogenized surface layer harder than that corresponding to 700 Brinell.

12. The method of hardening ferrous material which comprises adjusting the content of aluminum only in the surface layer of the material so that a hard structure of nitrogen-containing material will be formed in the layer by heating to predetermined temperatures in the presence of a substance that will yield nitrogen thereto, and then heating the material in the presence of nitrogen-yielding material.

13. The method of hardening ferrous material which comprises adjusting the content of aluminum only in the surface layer of the material so that a hard structure of nitrogen-containing material will be formed by heating to temperatures not exceeding 580° C. in the presence of a substance that will yield nitrogen thereto, and then heating the material to said temperatures in the presence of nitrogen-yielding material.

14. An article composed of a ferrous alloy, the surface layer of said alloy containing nitrogen and aluminum, the aluminum being present in a critical amount which will produce a hard nitrogen-containing substance corresponding to at least 700 Brinell by heating to temperatures of about 500° C. in the presence of ammonia, the core being free from aluminum in amounts which will produce said hard nitrogen-containing substance at said temperatures.

In testimony whereof I affix my signature.

AUGUSTUS B. KINZEL.